

June 16, 1936.

V. DIETZ

2,044,156

PRINTING

Filed Jan. 6, 1933

Fig. 1.



Fig. 2.



Fig. 3.



Fig. 4.



Fig. 5.



Fig. 6.



Fig. 7.



Fig. 8.



Fig. 9.



Fig. 10.



Fig. 11.



Inventor:

Valentin Dietz  
By Walter M. Fuller  
atty

Patented June 16, 1936

2,044,156

# UNITED STATES PATENT OFFICE

2,044,156

## PRINTING

Valentin Dietz, Cologne, Germany, assignor to  
Erwin B. Elliott and Maurice C. Boyd, Miami,  
Fla.

Application January 6, 1933, Serial No. 650,381  
In Germany October 11, 1932

### 7 Claims. (Cl. 41—41.5)

My present invention pertains to improvements and betterments in the methods and processes of printing from gelatin and analogous films or strata, and, among other things, aims to increase 5 the number of prints which can be secured from such gelatinous members, to improve the quality of the printed matter, to make the procedure so simple that inexperienced persons can perform it with facility and success, and to provide a method 10 which can be practised at small cost and with a simple printing mechanism or even by hand.

In the accompanying drawing the present invention has been illustrated more or less dia- 15 grammatically, and in this drawing—

Figure 1 shows the soaking of the gelatin film in a bath of glycerine, water, oxgall, para-phenylenediamine, and urotropine;

Figure 2 illustrates the film removed from the bath and its surface dried;

Figure 3 illustrates a sheet of paper bearing on its surface the image to be printed in a material capable of tanning the gelatin;

Figure 4 shows the paper applied to the surface of the gelatin;

Figure 5 shows the gelatin film with the paper removed and the gelatin film tanned;

Figure 6 shows the inking of the printing surface of the tanned film;

Figure 7 illustrates the printing operation;

Figure 8 presents a modified way of applying the gelatin tanning medium;

Figure 9 shows the process carried out in connection with the dry gelatin film;

Figure 10 shows the swelling of the gelatin film thus treated; and

Figure 11 sets forth another way of practising the process.

The present preferred performance comprises soaking a dry, gelatin-coated, celluloid film in a 40 bath of glycerin, water, and bile or ox-gall in the approximate proportion by weight of 75% pure glycerine, 24% water, and 1% bile or ox-gall, concentrated to a strength of about 75% solids, at which concentration such bile or ox-gall is in the 45 form of a sticky paste, but it is to be understood that it can be employed in powdered form if preferred, account of course being taken of its greater concentration.

The coated film is allowed to remain in such 50 bath for about 15 minutes, the period, of course, depending upon the temperature of the bath, whereupon it is withdrawn from the bath and the excess solution removed from the gelatin surface (see Figure 2), but such surface drying does not 55 eliminate the swelled characteristics of the gelatin

which have been brought about by the action of the glycerine and water.

Stated somewhat differently, the treated gelatin stratum although swollen and containing water, may be said to have a dry surface as distinguished from other swollen gelatins which are used for printing with wetted surfaces.

Instead of using a gelatin coating, a similar stratum of albumen, agar-agar, or other equivalent colloidal or gelatinous substance capable of 10 swelling in water may be used, and the backing or support instead of being celluloid may be waterproof-paper, glass, or any other suitable medium, which may be transparent, translucent, or opaque, although I have found in practice that 15 a white celluloid film is the best choice because it readily discloses an undesired ink smear thereon when taken up for use.

Hereinafter the term "gelatinous" has been used to designate any of the specified materials or 20 their equivalents.

The matter to be reproduced is written or printed 25 or otherwise applied to a sheet of paper or its equal by means of an ink containing an ingredient which has the capacity for tanning, shrinking, hardening, rendering water-insoluble or water non-distensible those parts of the swollen film with which it comes in contact (see Figure 3).

The term "tanning" used below in reference to 30 the gelatine is intended to have the meaning that the gelatin is modified in the stated manner immediately above referred to.

Almost all metal salts can be used for this tanning purpose, including iron chloride, which is 35 particularly powerful for accomplishing this result, especially due to the facility with which it penetrates to the base of the gelatine stratum, but such chloride cannot well be used in some cases because it is excessively corrosive.

Nitrates and sulfates in general are preferred; 40 for example, alum or aluminum sulfate may be employed to about 5% to 10% by weight of the water-soluble ink used, and in case a nitrate is employed, it is desirable to use about 5% of the weight of the ink. Tannin is also a gelatin-fixing 45 agent, but it has some tendency to spread. If it is employed alone, it would be used in about the proportion first indicated above.

My present preferred ink, however, for use on 50 a typewriter ribbon is approximately by weight as follows: aluminum sulfate 62.5%, mineral oil 23.4%, tannin 9.4%, carbon black 4.7%.

Iron sulfate or chrome alum, if employed, 55 would be used in about the same percentage,

and all of such salts should be used in a normal crystallized form.

Such style of ink may be availed of in any approved manner, for instance, as the ink of an inked ribbon on a typewriter, or the gelatin-fixing agent or agents may be employed as ingredients of the dry coating of a typewriter paper ribbon or sheet through which the printing is accomplished, or the needed fixing chemical may be used in any other way to reach the desired result.

The matter to be reproduced having been thus written or printed on a sheet of paper, the face of the latter displaying such matter is applied to and pressed on the unwetted surface of the swollen gelatin stratum (see Figure 4), and in a short time, say two or three minutes, more or less, the specified fixing agent or agents will have caused those portions of the gelatin layer which it or they have contacted to become tanned, hard, firm, and water-insoluble, and also incapable of being swollen in water, and the paper is removed from the face of the gelatin (see Figure 5).

25 Stated in other words, the one or more fixing or hardening ingredients shrink or condense the portions of the gelatin layer with which they come in contact, thus forming a somewhat depressed image in the surface of the gelatin.

30 The glycerine-water-bile mixture makes the gelatin layer ink repellent throughout its thickness, but the former ink-repellent quality of those parts of such layer as have been hardened and shrunk by the one or more fixing ingredients is overcome or neutralized so that such parts will readily accept the printing ink when applied thereto.

35 The dry or unwetted surface of such swollen stratum is then inked, the ink clinging to the hardened and set portions of it, but being repelled by the other parts so that the ink does not cleave to them (see Figure 6).

40 Then this inked, unwetted, swollen gelatin layer is used as a printing element, and, when a sheet of paper is pressed on it by hand or by machine, the ink on the gelatin surface is transferred to the paper as in the usual printing operation (see Figure 7), whereby the printed sheet is an exact reproduction of the original sheet printed with the specially-prepared ink.

45 The glycerine and water mixture which swells the gelatin also acts in a measure as an ink repellent, as does the bile or ox-gall, but one particularly advantageous feature of the bile is that it so toughens the swollen gelatin that many prints may be taken therefrom without injury to the gelatin stratum, and such toughening does not substantially reduce or diminish the swollen properties of the layer.

50 Instead of using the bile or ox-gall with glycerine and water, it may be employed with glycol as a swelling agent, in which case the mixture would be approximately by weight: glycol 99%, bile or ox-gall 1% (75% solids).

55 One of the particular advantages of this process resides in the fact that there is no necessity for wetting the surface of the swollen gelatin layer or resoaking it in water and/or glycerine or glycol during the printing operation, and for that reason a lighter pressure and a thinner ink can be used than has heretofore been customary in similar processes.

60 It has been discovered that, due to the continued application of the inking-roller over the unwetted surface of the gelatin stratum, and by

reason of the repeated pressing of the print paper on the gelatin surface, the bile, ox-gall, or its equivalent which contributes substantially to the ink-repellency of the gelatin is gradually and progressively removed or abstracted from the gelatin.

65 Even though this increasing or developing surface depletion or exhaustion of the incorporated ink-repellent bile may in a measure be overcome or replaced by the ink-repellent in the body of the gelatin layer working its way to the surface, it has been found that it is desirable to replace such abstracted or withdrawn material continuously to permit it to be present in the gelatin film at all times substantially in its full or required amount.

70 This result can be readily and easily accomplished by properly charging the ink with a suitable amount of the ink-repellent bile or ox-gall, and a convenient and appropriate mixture would be weight as follows: lamp-black about 22%, medium-consistency linseed-oil-varnish approximately 66%, and ox-gall 12% (75% solids).

75 The amount of such incorporated ink-repellent to be used in the ink cannot always be stated with accuracy because the quantity to be mixed in the ink depends in material measure upon the nature and quality of the color employed and upon the grade and consistency of the linseed-oil-varnish.

80 The correct proportion of such ink-repellent to be mixed or combined with the ink can, however, be comparatively easily determined by simple tests, bearing in mind that if too little is used the gelatin layer will be gradually starved of its repellent, which effect will be indicated by the character of the prints; whereas if too much is put in the ink, the ink will not properly adhere to those sections of the gelatin layer to which it should cleave.

85 Thus, for each application of ink, a suitable supply of the ink-repellent is simultaneously made to the surface of the gelatin stratum, which either prevents the withdrawal of such repellent from the gelatin or replaces that which may be abstracted, but, in either case, the result is the same in that the gelatin is at all times in proper condition for printing and does not become exhausted or deprived of any of its essential constituents.

90 The ink-repellent used acts not only to make the condition of the gelatin such that it will not receive the ink, but it also renders the swollen gelatin layer firmer and tougher than has heretofore been possible, and, accordingly, such gelatin stratum can be used for producing a large number of prints of the highest quality. Seemingly, both the glycerine or glycol and the bile or ox-gall tend to give the swollen portions of the gelatin substantially improved wearing qualities without impairing its swollen characteristics.

95 As stated above, the employment of the ink-repellent, bile or ox-gall, makes the swollen gelatin stratum tougher and harder, and it may also be remarked that this particular ink-repellent reduces the stickiness or adhesiveness of the gelatin surface, thus lessening the tendency to withdraw or abstract the repellent from the gelatin during the printing operation.

100 Stated somewhat differently, the use of the repellent bile or ox-gall tends to maintain the surface of the gelatin comparatively smooth, whereas as by the old wet process there is a distinct tendency to cause it to become somewhat rough.

The specified bile or ox-gall when incorporated in the ink has the further advantage of causing the ink to dry and harden rapidly, so that danger of smearing the prints is overcome.

5 The preferred procedure set forth in detail above is one ordinarily employed where a considerable number of prints is required, but, in those cases where a comparatively small number of prints suffices, the ink-repellent may be 10 incorporated in the gelatin stratum alone or in the ink alone.

The most available form of bile is the well-known ox-gall, the principal ingredients of which are sodium glycocholate and sodium taurocholate, and while it is somewhat difficult and more or less expensive to separate such salts from one another completely, I have found that sodium glycocholate is apparently substantially more effective than the sodium taurocholate in the performance of the ink-repellent function, and, therefore, it may be advisable or desirable to use such sodium glycocholate rather than the cheaper ox-gall.

Again, instead of using the specified bile or ox-gall, one or more dry bile salts may be employed, account of course being taken of the fact that a correspondingly different quantity would be required because of the dry form used.

In order to increase the intensity of the gelatin-fixing when an inked ribbon is employed, about one to two per cent of urotropine may be added to the repellent in the gelatin layer or may be wiped over the surface of the gelatin stratum, and when it comes in contact with an acid salt it breaks down into ammonia and formaldehyde, the latter being an intense hardening agent (see Figure 1).

Instead of incorporating the gelatin fixing or setting ingredient in the ink employed in printing the master sheet which is subsequently applied to the swollen gelatin surface, the printing may be done on such sheet with any suitable medium which remains fresh or moist at least temporarily, and then the gelatin fixing or setting agent in the form of a powder may be sprinkled over such printed matter to which it adheres (see Figure 8), and then such sheet is transferred to the gelatin surface as indicated hereinbefore.

50 As a modification of this process, but not quite so simple as the method described above, the original gelatin layer may be swollen with glycerine and water, or with glycol, and then after the gelatin stratum has been tanned or set by the matter to be printed, either the layer may be soaked in a bath containing any of the above specified ink-repellents, the excess removed from the surface, and the printing performed as indicated above; or the ink containing the ink-repellent may be used on the swollen layer without such soaking, or both of these procedures may be employed conjointly.

In some instances, it may be feasible to apply the matter to be printed with any one or more of the specified gelatin-fixing chemicals to the surface of a gelatin stratum dry throughout its thickness, either directly or first on a sheet of paper which is then pressed on the surface (see Figure 9), and then swelling the stratum, as, for example, by the use of steam (see Figure 10), and thereupon proceeding as indicated above.

If desired, such original bone-dry stratum may have any one or more of the ink-repellent agents incorporated in it before the gelatin-fixing operation takes place.

In some cases where the fixing of the completely dry stratum takes place it may be desirable to wipe over the surface of the gelatin layer with water before it is subjected to the further use of a moistening agent.

Still another way of employing the invention is to cut the matter to be reproduced in a typewriter without an ink-ribbon in a wax or other appropriate stencil, so that the typewritten letters cut through the wax or its equivalent.

Then such stencil is laid on the surface of the swollen gelatin layer containing the one or more bile salts and an absorbent sheet impregnated with full strength formaldehyde is superposed on top of the stencil and rolled or pressed thereon so 15 that the formaldehyde acting on the underlying gelatin through the cut matter of the stencil tans, sets, or hardens such portions only of the gelatin (see Figure 11).

Thereupon, the absorbent sheet and the stencil 20 are removed and the gelatin layer used for printing, as indicated above.

By this procedure the wax or the like of the stencil prevents the action of the setting formaldehyde from spreading, with the result that 25 well-defined, clear-cut letters are fixed in the gelatin.

Of course, such original gelatin layer need not necessarily be impregnated with the one or more bile salts, as they may be used solely in the ink, 30 if preferred, or their use may in some cases be dispensed with.

The term "ink-repellent" as herein applied to the bile, ox-gall, or bile salts has been employed with the meaning that the specified material 35 performs the function of augmenting or reenforcing the capacity of the swollen gelatin stratum to reject the applied ink and to preserve and to prolong indefinitely the property of the distended gelatin to repel the ink, thus permitting the gelatin stratum to be used with its unwetted surface during any printing operation and over the entire service period of the layer.

The invention, as specified in the following claims, is not restricted to the precise details of 45 procedure set forth hereinabove, and those skilled in this art will readily appreciate that more or less major and minor modifications may be resorted to.

For example, when any of the foregoing processes are practiced under somewhat dry or warm atmospheric conditions, it is desirable to use an amine, such as ethylenediamine, para-phenylenediamine, or alpha-naphthylamine, as an ingredient of the water-glycerine-bile bath solution 55 (see Figure 1), or it may be applied to the surface of the galatinous layer before inking (so that it will be absorbed by such surface), or it may be employed as an ingredient of the ink. In the first instance, one-quarter of one per cent 60 is added to the water-glycerine-bile solution, or in the second example approximately one-quarter of one per cent solution is used for the surface application, or in the third case about one per cent is added to the ink, all of these proportions 65 being by weight. If preferred, the amine may be used both in association with the gelatin and in the ink.

I prefer to use alpha-naphthylamine or ethylenediamine in the film because para-phenylene-diamine gives the film a yellowish color.

I claim:

1. In the art of printing, swelling a suitably-supported gelatinous layer and at the same time making the layer ink-repellent by an agent other 75

than the swelling medium but incorporated in said medium and including an amine, and by a tanning medium tanning the parts of such layer in agreement with the image to be printed.

5. 2. In the art of printing, swelling a suitably-supported gelatinous layer and at the same time making the layer ink-repellent by an agent other than the swelling medium but incorporated in said medium and including an amine, and tanning the parts of such layer in agreement with the image to be printed by a tanning medium incorporating iron chloride.

15. 3. In the art of printing, swelling a suitably-supported gelatinous layer and at the same time making the layer ink-repellent by an agent other than the swelling medium but incorporated in said medium and including an amine, and tanning the parts of said layer in agreement with the image to be printed by a tanning medium incorporating iron chloride and urotropine.

20. 4. In the art of printing, swelling a suitably-supported gelatinous layer and at the same time making the layer ink-repellent by an agent other than the swelling medium but incorporated in said medium and including an amine, and tanning the parts of said layer in agreement with the image to be printed by a tanning medium incorporating aluminum sulfate.

5. In the art of printing, swelling a suitably-supported gelatinous layer and at the same time making the layer ink-repellent by an agent other than the swelling medium but incorporated in said medium and including an amine, and tanning the parts of said layer in agreement with the image to be printed by a tanning medium incorporating aluminum sulfate and urotropine.

10. 6. In the art of printing, swelling a suitably-supported gelatinous layer and at the same time making the layer ink-repellent by an agent other than the swelling medium but incorporated in said medium and including an amine, and tanning the parts of said layer in agreement with the image to be printed by a tanning medium incorporating alum.

15. 7. In the art of printing, swelling a suitably-supported gelatinous layer and at the same time making the layer ink-repellent by an agent other than the swelling medium but incorporated in said medium and including an amine, and tanning the parts of said layer in agreement with the image to be printed by a tanning medium incorporating alum and urotropine.

20. VALENTIN DIETZ.

25.